



US008896405B2

(12) **United States Patent**  
**Hachiya et al.**

(10) **Patent No.:** **US 8,896,405 B2**  
(45) **Date of Patent:** **Nov. 25, 2014**

(54) **COIL-TYPE ELECTRONIC COMPONENT**

(71) Applicant: **Taiyo Yuden Co., Ltd.**, Tokyo (JP)

(72) Inventors: **Masahiro Hachiya**, Takasaki (JP);  
**Atsushi Tanada**, Agatsuma-gun (JP);  
**Kenji Otake**, Takasaki (JP); **Kiyoshi Tanaka**, Agatsuma-gun (JP); **Tetsuyuki Suzuki**, Agatsuma-gun (JP)

(73) Assignee: **Taiyo Yuden Co., Ltd.**, Tokyo (JP)

(\*) Notice: Subject to any disclaimer, the term of this patent is extended or adjusted under 35 U.S.C. 154(b) by 0 days.

(21) Appl. No.: **13/662,035**

(22) Filed: **Oct. 26, 2012**

(65) **Prior Publication Data**

US 2013/0120097 A1 May 16, 2013

(30) **Foreign Application Priority Data**

Oct. 28, 2011 (JP) ..... 2011-236947

(51) **Int. Cl.**

**H01F 5/00** (2006.01)  
**H01F 17/04** (2006.01)  
**H01F 27/28** (2006.01)  
**H01F 27/24** (2006.01)  
**H01F 27/02** (2006.01)  
**H01F 1/40** (2006.01)  
**H01F 1/33** (2006.01)  
**H01F 1/24** (2006.01)

(52) **U.S. Cl.**

CPC .. **H01F 1/40** (2013.01); **H01F 1/33** (2013.01);  
**H01F 1/24** (2013.01); **H01F 17/045** (2013.01)  
USPC ..... **336/200**; 336/221; 336/232; 336/233;  
336/83

(58) **Field of Classification Search**

USPC ..... 336/200, 221, 232, 233, 234, 83  
See application file for complete search history.

(56) **References Cited**

U.S. PATENT DOCUMENTS

4,129,444 A 12/1978 Dreyer et al.  
5,352,522 A 10/1994 Kugimiya et al.  
5,522,946 A 6/1996 Tomita et al.  
6,392,525 B1 5/2002 Kato et al.

(Continued)

FOREIGN PATENT DOCUMENTS

CN 101308719 A 11/2008  
CN 101927344 A 12/2010

(Continued)

Primary Examiner — Alexander Talpalatski

Assistant Examiner — Kazi Hossain

(74) Attorney, Agent, or Firm — Law Office of Katsuhiro Arai

(57) **ABSTRACT**

A coil-type electronic component having a coil inside or on the surface of a base material, characterized in that the base material of the coil-type electronic component is constituted by a group of soft magnetic alloy grains whose main ingredients are iron, silicate and chromium, and that an oxide layer is formed on the surface of each soft magnetic alloy grain, where the oxide layer is produced as a result of oxidization of the grain and has more chromium than the alloy grain, and this oxide layer has a two-layer structure constituted by an inner layer whose main ingredient is chromium oxide and an outer layer whose main ingredient is iron-chromium oxide, and the outer layers of soft magnetic alloy grains are inter-bonded.

**5 Claims, 5 Drawing Sheets**



| (56)              | References Cited                    | FOREIGN PATENT DOCUMENTS  |
|-------------------|-------------------------------------|---------------------------|
|                   | U.S. PATENT DOCUMENTS               |                           |
| 6,764,643 B2      | 7/2004 Sagawa et al.                | CN 102007549 A 4/2011     |
| 6,784,782 B2      | 8/2004 Inoue et al.                 | JP H04-346204 A 12/1992   |
| 6,814,928 B2      | 11/2004 Sagawa et al.               | JP 07-201570 A 8/1995     |
| 7,422,697 B2      | 9/2008 Takahashi et al.             | JP H09-074011 A1 3/1997   |
| 7,446,638 B2      | 11/2008 Nogi                        | JP 2000-030925 A1 1/2000  |
| 8,018,313 B2      | 9/2011 Tada et al.                  | JP 2001-011563 A1 1/2001  |
| 8,416,051 B2 *    | 4/2013 Matsuura et al. .... 336/233 | JP 2001-118725 A1 4/2001  |
| 2004/0140016 A1   | 7/2004 Sakamoto et al.              | JP 2002-305108 A1 10/2002 |
| 2004/0209120 A1   | 10/2004 Inoue et al.                | JP 2002-313620 A1 10/2002 |
| 2007/0290161 A1   | 12/2007 Tokuoka et al.              | JP 2002-343618 A1 11/2002 |
| 2008/0003126 A1   | 1/2008 Watanabe et al.              | JP 2005-286145 A 10/2005  |
| 2008/0012679 A1   | 1/2008 Okabe et al.                 | JP 2007-019134 A1 1/2007  |
| 2008/0029300 A1 * | 2/2008 Harada et al. .... 174/391   | JP 2007-027354 A 2/2007   |
| 2008/0061264 A1   | 3/2008 Maeda et al.                 | JP 2007-027354 A1 2/2007  |
| 2008/0152897 A1   | 6/2008 Maeda et al.                 | JP 2007-123703 A1 5/2007  |
| 2008/0231409 A1   | 9/2008 Kugai et al.                 | JP 2007-258427 A 10/2007  |
| 2008/0278273 A1 * | 11/2008 Lee et al. .... 336/83      | JP 2007-299871 A1 11/2007 |
| 2009/0045905 A1   | 2/2009 Nakagawa et al.              | JP 2008-028162 A1 2/2008  |
| 2009/0102589 A1 * | 4/2009 Lee et al. .... 336/83       | JP 2008-041961 A1 2/2008  |
| 2010/0253463 A1   | 10/2010 Shimomura et al.            | JP 2008-195986 A1 8/2008  |
| 2010/0289609 A1 * | 11/2010 Liao et al. .... 336/221    | JP 2009-010180 A 1/2009   |
| 2011/0024670 A1   | 2/2011 Otsuki et al.                | JP 2009-088496 A1 4/2009  |
| 2011/0025444 A1 * | 2/2011 Sugiyama et al. .... 336/212 | JP 2009-088502 A1 4/2009  |
| 2011/0133881 A1   | 6/2011 Nakajima et al.              | JP 2009088502 * 4/2009    |
| 2011/0227690 A1 * | 9/2011 Watanabe et al. .... 336/221 | TW 2011-249774 A1 12/2011 |
| 2011/0267167 A1 * | 11/2011 Ogawa et al. .... 336/221   | TW 200845057 A 11/2008    |
| 2012/0038449 A1   | 2/2012 Ogawa et al.                 | TW M388724 U1 9/2010      |
| 2012/0070567 A1   | 3/2012 Watanabe et al.              | WO 2009/001641 A1 12/2008 |
|                   |                                     | WO 2009/128425 A1 10/2009 |
|                   |                                     | WO 2010/013843 A1 2/2010  |

\* cited by examiner

Fig. 1



Fig. 2



Fig. 3



Fig. 4



Fig. 5



Fig. 6



Fig. 7



$$\sigma_b = \frac{M}{I} \times \frac{h}{2} = \frac{3WL}{2bh^2}$$

Width of test piece:  $b$  (mm)  
Thickness of test piece:  $h$  (mm)  
3-point bending rupture stress ( $\sigma_b$ )

Fig. 8

Electrode Layout in Resistivity Test

## COIL-TYPE ELECTRONIC COMPONENT

## BACKGROUND

## 1. Field of the Invention

The present invention relates to a coil-type electronic component, and more specifically to a coil-type electronic component using a soft magnetic alloy, suitable for a compact coil-type electronic component that can be surface-mounted on a circuit board.

## 2. Description of the Related Art

Magnetic cores of choke coils used in high-frequency applications are traditionally ferrite cores, cores cut from thin metal sheets, and powder-compressed magnetic cores. Use of metal magnetic materials has an advantage over ferrites, as these materials can achieve high saturated magnetic flux densities. However, metal magnetic materials are poor in insulation property and must be given insulation treatment. Patent Literature 1 proposes mixing a Fe—Al—Si powder having surface oxide film with a binder, compression-molding the mixture, and then heat-treating the molded product in an oxidizing ambience. According to the patent literature, heat-treating the molded product in an oxidizing ambience has the effect of forming an oxide layer (alumina) in those areas of the insulation layer on the surface of the alloy powder that have broken during compression molding, thereby achieving a complex magnetic material offering good direct-current superimposition characteristics with minimal core loss. Patent Literature 2 describes laminating a metal magnetic layer formed by a metal magnetic paste which contains metal magnetic grains as the main ingredient, and also glass, with a conductive pattern formed by a conductive paste containing silver or other metal, and then baking the obtained laminated electronic component, which has the coil pattern formed in the laminate, at a temperature of 400° C. or above in a nitrogen ambience.

## PATENT LITERATURES

[Patent Literature 1] Japanese Patent Application Laid-open No. 2001-11563

[Patent Literature 2] Japanese Patent Application Laid-open No. 2007-27354

## SUMMARY

The complex magnetic material in Patent Literature 1 requires a high pressure during compression molding because the Fe—Al—Si powder used for molding has an oxide film formed on its surface beforehand. This material also presents another problem in that, when it is applied to a power inductor or other electronic component through which higher current must flow, further size reduction cannot be fully supported. On the other hand, the laminated electronic component proposed in Patent Literature 2 is a laminated electronic component using a metal magnetic layer which is formed by a metal magnetic paste that contains metal magnetic grains as the main ingredient, and also glass. Although the resistance improves due to the glass layer, the fill ratio of the metal magnetic material drops due to the mixing of glass and the magnetic permeability  $\mu$  and other magnetic characteristics also drop.

The present invention was developed in light of the aforementioned situation and the object of the present invention is to provide a coil-type electronic component that can be produced at low cost and comprises a magnetic material offering higher magnetic permeability and higher saturated magnetic

flux density at the same time, as well as a method of manufacturing such coil-type electronic component.

Any discussion of problems and solutions involved in the related art has been included in this disclosure solely for the purposes of providing a context for the present invention, and should not be taken as an admission that any or all of the discussion were known at the time the invention was made.

After studying repeatedly in earnest to achieve the aforementioned object, the inventors of the present invention found that, by mixing with a binder and molding soft magnetic alloy grains whose main ingredients are iron, silicate and chromium and then heat-treating the molded product in an oxygen-containing ambience under specific conditions, an oxide layer having a two-layer structure would be formed on the surface of the heat-treated metal grains, and this oxide layer would cause the alloy grains to bond together, where, of the oxide layers in the two-layer structure, the inner layer formed by an oxide layer whose main ingredient is chromium oxide would cover the soft magnetic alloy grains to prevent promotion of oxidization in the soft magnetic alloy grains while suppressing deterioration in characteristics. It was also revealed that the outer layer of the two-oxide-layer structure is formed as an oxide layer whose main component is iron-chromium oxide which is thicker than the aforementioned inner layer, and therefore insulation property could be improved. Furthermore, it was found that, because the surface oxide layer not involved in the inter-bonding of alloy grains has irregularities and the specific surface area of grains increases after the heat treatment, insulation property would improve further.

The present invention was completed based on the aforementioned findings, and is described as follows:

<1> A coil-type electronic component having a coil inside or on the surface of a base material, wherein said coil-type electronic component is characterized in that the base material is constituted by a group of soft magnetic alloy grains whose main ingredients are iron, silicate and chromium, and in that an oxide layer having a two-layer structure is formed on the surface of each soft magnetic alloy grain where, of the oxide layers in the two-layer structure, the inner layer is primarily constituted by chromium oxide while the outer layer is primarily constituted by iron-chromium oxide, and the outer layers on soft magnetic alloy grains are inter-bonded.

<2> A coil-type electronic component according to <1>, characterized in that, of the oxide layers in the two-layer structure, the outer layer is thicker than the inner layer.

<3> A coil-type electronic component according to <1> or <2>, characterized in that the surface of the outer oxide layer not bonding the soft magnetic alloy grains together has irregularities.

<4> coil-type electronic component according to any one of <1> to <3>, characterized in that the base material has the soft magnetic alloy grains inter-bonded not via the oxide layers.

According to the present invention, a thick oxide layer can be formed on the outer side of a conventional oxide layer formed on the alloy grain surface and having a high chromium content, where this outer layer has higher specific resistance than the conventional oxide layer and is primarily constituted by iron-chromium oxide, by suitably heat-treating the soft magnetic alloy grains whose main ingredients are iron, silicate and chromium, and consequently insulation property can be improved. In addition, as the soft magnetic alloy grains are coated with the inner layer constituted by an oxide layer whose main ingredient is chromium oxide, excessive promotion of oxidization in the soft magnetic alloy

grains can be prevented and deterioration of characteristics can be suppressed. Furthermore, the heat treatment under the present invention produces irregularities on the grain surface and increases the specific area, which in turn achieves the inter-bonding of alloy grains demonstrated by prior art to improve  $\mu$ , while at the same time the irregularities of the surface oxide layer not bonding the alloy grains increase the surface resistance and thereby improve the insulation property further.

For purposes of summarizing aspects of the invention and the advantages achieved over the related art, certain objects and advantages of the invention are described in this disclosure. Of course, it is to be understood that not necessarily all such objects or advantages may be achieved in accordance with any particular embodiment of the invention. Thus, for example, those skilled in the art will recognize that the invention may be embodied or carried out in a manner that achieves or optimizes one advantage or group of advantages as taught herein without necessarily achieving other objects or advantages as may be taught or suggested herein.

Further aspects, features and advantages of this invention will become apparent from the detailed description which follows.

#### BRIEF DESCRIPTION OF THE DRAWINGS

These and other features of this invention will now be described with reference to the drawings of preferred embodiments which are intended to illustrate and not to limit the invention. The drawings are greatly simplified for illustrative purposes and are not necessarily to scale.

FIG. 1 is a side view showing a first embodiment of a base material using a soft magnetic alloy for an electronic component conforming to the present invention.

FIG. 2 is a schematic view illustrating an oxide layer model constituted by a two-layer structure formed according to the preset invention.

FIG. 3 is a side view, with partial perspective projection, of the first embodiment of a coil-type electronic component under the present invention.

FIG. 4 is a longitudinal section view showing the internal structure of the coil-type electronic component in the first embodiment.

FIG. 5 is a perspective view of internal structure, showing an example of variation of the embodiment of base material using a soft magnetic alloy for an electronic component conforming to the present invention.

FIG. 6 is a perspective view of internal structure, showing an example of variation of the embodiment of an electronic component under the present invention.

FIG. 7 is an explanation drawing showing how samples were measured for 3-point bending rupture stress in examples of the present invention.

FIG. 8 is an explanation drawing showing how samples were measured for volume resistivity in examples of the present invention.

#### DESCRIPTION OF THE SYMBOLS

- 1: Grain
- 2: Inner layer of an oxide layer
- 3: Outer layer of an oxide layer
- 10, 10': Base materials using a soft magnetic alloy for an electronic component
- 11: Drum-type core
- 11a: Winding center
- 11b: Flange part

- 12: Sheet-shaped core
- 14: External conductive film
- 14a: Baked conductive film layer
- 14b: Ni plating layer
- 14c: Sn plating layer
- 15: Coil
- 15a: Winding part
- 15b: End (joined part)
- 20: Electronic component (winding-type chip inductor)
- 31: Laminated chip
- 34: External conductive film
- 35: Internal coil
- 40: Electronic component (laminated chip inductor)

#### DETAILED DESCRIPTION OF EMBODIMENTS

In the present disclosure, “an oxide layer formed as a result of oxidation of the grain” refers to an oxide layer formed by oxidation greater than natural oxidation of the grain, which 20 oxide layer is an oxide layer grown by reacting a surface of the grain and oxygen by heat treatment of a molded body formed from grains in an oxidizing atmosphere. Also, a “layer” refers to a layer distinguishable from others based on its compositions, structures, properties, appearance, and/or production 25 processes, etc., including a layer having a discrete or unclear boundary, and a layer which is a continuous film on the surface of a grain or which is a film having partially a discontinued portion. In some embodiments, an “oxide layer” is a continuous film covering the entire surface of each grain. 30 Further, such an oxide layer possesses any of the characteristics identified in the present disclosure, and the oxide layer grown by oxidation of the grain surface can be distinguished from an oxide film formed by other methods. In the present disclosure, relative terms such as “greater”, “easier”, etc. 35 refer to substantial differences by degrees which cause significant differences in function, structure, or effect/result.

In some embodiments, “a soft magnetic alloy whose main elements are iron, silicon, and chrome” or the like refers to a soft magnetic alloy constituted by compositions consisting 40 essentially of or consisting of iron, silicon, and chrome (other than impurities), “an inner layer whose main element is chromium oxide” refers to an inner layer formed by oxidization of the soft magnetic alloy wherein chromium oxide is the main oxide, and “an outer layer whose main elements are iron oxide and chromium oxide” refers to an outer layer formed by 45 oxidization of the soft magnetic alloy wherein iron oxide and chromium oxide are the main oxide. In some embodiments, “an inner layer whose main element is chromium oxide” and “an outer layer whose main elements are iron oxide and 50 chromium oxide” refer to compositions wherein the inner layer contains more chromium oxide than the outer layer, and the outer layer contains more iron oxide than the inner layer. In some embodiments, the inner layer and the outer layer do not have a clear boundary and the compositions of the inner 55 layer and the outer layer change continuously along the depth direction, wherein the inner layer and the outer layer are defined as different layers, any point of each layer satisfying the above compositional definitions.

The following explains a first embodiment of a base material using a soft magnetic alloy for an electronic component conforming to the present invention, by referring to FIGS. 1 to 4. FIG. 1 is a side view showing the exterior of a base material 10 using a soft magnetic alloy for the electronic component in this embodiment. The base material 10 using a soft magnetic alloy for the electronic component in this embodiment is used as a core around which a coil of a coil-type chip inductor is wound. The drum-type core 11 has a sheet-shaped winding

center **11a** which is provided in parallel with the mounting surface of a circuit board, etc., and around which a coil is wound, and a pair of flange parts **11b**, **11b** provided at the opposing ends of the winding center **11a**, which has a drum-type appearance. Coil ends are electrically connected to a conductive film **14** formed on the surface of flange parts **11b**, **11b**.

The base material **10** using a soft magnetic alloy for electronic components, as proposed by the present invention, is constituted by a group of soft magnetic alloy grains whose main ingredients are iron (Fe), silicate (Si) and chromium (Cr), where formed on the surface of each soft magnetic grain is a layer of metal oxide having a two-layer structure, produced by heat-treating the grain suitably in an oxygen-containing ambience and thereby oxidizing the grain (hereinafter referred to as "oxide layer"). The remainder of the Specification uses specific names or symbols to refer to the elements.

FIG. 2 is a schematic view of a simplified model comprising two soft magnetic alloy grains with the aim of explaining the oxide layer model having a two-layer structure, as proposed by the present invention, in an easy-to-understand manner. In the figure, **1** indicates the soft magnetic alloy grain, **2** indicates the inner oxide layer, and **3** indicates the outer oxide layer, respectively. The oxide layers are produced on the surface of the grain as a result of oxidization of the grain, and have higher chromium contents than the alloy grain. The oxide layers constitute a two-layer structure in that there are the inner layer **2** whose main ingredient is chromium oxide, and the outer layer **3** which is present on the outer side of the inner layer and whose main ingredient is iron-chromium oxide offering higher specific resistance. The outer layer **3** is formed thicker than the inner layer **2**, and the surface of the soft magnetic alloy grain **1** is coated with the inner layer **2**, where the soft magnetic alloy grains **1** are inter-connected via their respective outer oxide layers **3** as shown in (A) of FIG. 2 or directly without involving any oxide layer as shown in (B) of FIG. 2. Furthermore, the outer oxide layer not involved in the inter-bonding of soft magnetic alloy grains has surface irregularities and the specific surface area of the grains is larger than before the heat treatment, which has the effect of improving the insulation property further. The coil-type electronic component thus achieved, which has a fine structure and uses soft magnetic alloy grains according to the present invention, exhibits superior characteristics to its conventional counterparts in terms of high magnetic permeability and high resistance.

The two-layer structure can be checked by polishing the target product to a mirror surface, applying ion milling (CP), and then observing it using a scanning electron microscope (SEM). The oxide layer can be identified as follows. First, the base material is polished in such a way that its cross-section cut along the center line in the thickness direction is exposed, and the obtained cross-section is captured at a magnification of 3000 using a scanning electron microscope (SEM) to obtain a composition image. The scanning electron microscope (SEM) composition image shows different constituent elements as contrast (brightness) differences. Next, the pixels of the composition image obtained above are classified into four brightness levels. The brightness levels are determined in such a way that, among the grains whose cross-section outline can be fully observed in the above composition image, a grain whose size, being calculated as the simple average D of the long-axis dimension d1 and short-axis dimension d2 of its cross-section, or  $D=(d1+d2)/2$ , is greater than the average grain size (d50%) of the material grain (material alloy grain on which no oxide layer is formed) is deemed to be of the reference brightness level of the composition contrast.

Accordingly, any portion corresponding to this brightness level in the above composition image is considered a grain **1**. Also, any portion whose composition contrast is one level darker than the aforementioned reference brightness level is considered an outer oxide layer **3**, while any portion whose brightness level is even darker is considered an inner oxide layer **2** (refer to the schematic view in FIG. 2). Desirably, measurement is taken multiple times. Any portion whose brightness level is darker than any of the aforementioned brightness levels is considered a void (not illustrated).

As for the thickness measurement of the inner oxide layer **2** and outer oxide layer **3**, the thickness of the inner layer **2** and that of the outer layer **3** can be obtained from the shortest distance from the boundary surface of the grain and the inner oxide layer **2**, to the boundary surface of the outer oxide layer **3** and the void. To be specific, the thickness of the oxide layer can be obtained as follows: A cross-section of the base material **10** in the thickness direction is captured using a SEM (scanning electron microscope) at a magnification of 1000 or 15 2000, and the center of gravity of one grain in the obtained composition image is obtained using imaging software, and line analysis is performed using an EDS (energy-dispersive X-ray spectrometer) from this center of gravity in the radial direction. An area whose oxygen concentration is at least 25 three times the oxygen concentration at the center of gravity is judged an oxide (this means that, considering the measurement error, three times is set as the threshold and an area whose oxygen concentration is less than three times the oxygen concentration at the center of gravity is judged a non-oxide layer, where the oxygen concentration of an actual oxide layer can be 100 times the oxygen concentration at the center of gravity or more), and the total thickness of two oxide layers, or namely the inner layer and outer layer, is measured as the length to the outer periphery of the grain. Here, the 30 thickness of the outer oxide layer **3** is obtained from the brightness difference as explained above, and the obtained thickness is subtracted from the total oxide layer thickness to arrive at the thickness of the inner oxide layer **2**. The total oxide layer thickness is the average thickness obtained as a 35 simple average of the maximum and minimum thicknesses of the oxide layer present on the surface of the grain **1** identified by the aforementioned method, from the surface of the grain **1**. The thickness of the outer oxide layer **3** is the average 40 thickness obtained as a simple average of the maximum and minimum thicknesses of the outer oxide layer **3** present on the surface of the inner oxide layer **2** identified by the aforementioned method, from the surface of the inner layer **2**.

Under the present invention, the thickness of the inner layer **2** and the outer layer **3** of the oxide layer can vary among grains. However, a preferred range of the inner layer **2** is 5 to 50 nm, and a preferred range of the outer layer **3** is 50 to 500 nm. The thickness of the oxide layer formed on the surface of a single alloy grain can vary from area to area. In an embodiment, alloy grains can be inter-bonded via oxide layers 55 thicker than those present on the alloy grain surface (oxide layers adjacent to voids) in order to achieve high strength as a whole. In another embodiment, alloy grains can be inter-bonded via oxide layers thinner than those present on the alloy grain surface (oxide layers adjacent to voids) in order to 60 achieve high magnetic permeability as a whole. In an embodiment, the average grain size of soft magnetic grains having the oxide layer is virtually or roughly the same as the average grain size of the material grain (grain before molding and heat treatment).

Under the present invention, the inner layer **2** of the aforementioned two-oxide-layer structure is an oxide layer whose main ingredient is chromium oxide, while the outer layer **3** is

an oxide layer whose main ingredient is iron-chromium oxide. This two-layer structure can be checked using an EDS (energy-dispersive X-ray spectrometer) and has the effect of suppressing the drop in saturated magnetic density.

The composition ratio of grains in the above base material using a soft magnetic alloy for an electronic component (hereinafter also referred to as "a soft magnetic alloy base material for an electronic component") can be checked as follows. First, a material grain is polished until its cross-section cutting across the center of the grain is exposed, and the obtained cross-section is captured with a scanning electron microscope (SEM) at a magnification of 3000 times to obtain a composition image, which is then used to calculate the composition near the center of the grain by the ZAF method through energy diffusion X-ray analysis (EDS). Next, the above base material using a soft magnetic alloy for an electronic component is polished until its cross-section in a thickness direction cutting across roughly the center of the base material is exposed, and the obtained cross-section is captured with a scanning electron microscope (SEM) at a magnification of 3000 times to obtain a composition image. Among the grains shown in this composition image whose cross-section outline can be fully observed, a grain is extracted, whose simple average size  $D=(d_1+d_2)/2$  is greater than the average grain size of material grains (d50%), where  $d_1$  and  $d_2$  represent the long-axis dimension and short-axis dimension of the cross-section of each grain, respectively, and the composition near the point of intersection of its long axis and short axis is calculated by the ZAF method through energy diffusion X-ray analysis (EDS). The result is then compared against the composition ratio in the above material grain to show the composition ratio in the alloy grain of the above base material using a soft magnetic alloy for an electronic component. (Since the composition of the material grain is known, by comparing the composition ratios determined by the ZAF method, the composition of the alloy grain can be determined.)

The base material **10** under the present invention has multiple soft magnetic alloy grains **1** and an oxide layer produced on the surface of each grain **1**, where the oxide layer has a two-layer structure constituted by an inner layer **2** and an outer layer **3**, and the soft magnetic alloy grain **1** has a composition of 2 to 8 percent by weight of chromium, 1.5 to 7 percent by weight of silicate, and 88 to 96.5 percent by weight of iron, where desirably the arithmetic mean size of soft magnetic grains is 30  $\mu\text{m}$  or less. The inner oxide layer **2** and outer oxide layer **3** contain at least chromium, where the peak intensity ratios of chromium to iron, R2 and R3, as measured by energy-dispersive X-ray spectrometry using a scanning electron microscope, are both virtually greater than the peak intensity ratio of chromium to iron, R1, in the grain. Also, while the main ingredient of the outer oxide layer is iron-chromium oxide, the main ingredient of the inner oxide layer is chromium oxide, which means that the peak intensity ratio of chromium to iron in the inner oxide layer **2**, or R2, is greater than the peak intensity ratio of chromium to iron in the outer oxide layer **3**, or R3. Furthermore, multiple grains partially have a void in between.

As for the aforementioned soft magnetic alloy base material for electronic components, the intensity ratio of chromium to iron in the grain **1**, or R1, peak intensity ratio of chromium to iron in the inner oxide layer **2**, or R2, and peak intensity ratio of chromium to iron in the outer oxide layer **3**, or R3, can be respectively obtained as follows. First, the composition of the point of intersection between the long axis  $d_1$  and short axis  $d_2$  in the grain **1** is obtained on the aforementioned composition image by SEM-EDS. Next, the total

thickness of the oxide layer on the surface of the grain **1**, and maximum thickness  $t_1$  and minimum thickness  $t_2$  of the outer layer **3**, are measured on the composition image. Each average thickness ( $T=(t_1+t_2)/2$ ) is obtained from the measured values, and the average thickness of the outer layer **3** is subtracted from the average total thickness of the oxide layer to arrive at the average thickness of the inner oxide layer **2**. Next, locations whose oxide layer thickness corresponds to the average thickness of the inner layer **2** or average thickness 10 of the outer layer **3** are identified, and the composition at the center point of the two locations is obtained by SEM-EDS. Thereafter, the peak intensity ratio of chromium to iron  $R1=C1_{CrKa}/C1_{FeKa}$  can be obtained from the iron intensity  $C1_{FeKa}$  and chromium intensity  $C1_{CrKa}$  in the grain **1**. Also, 15 the peak intensity ratio of chromium to iron  $R2=C2_{CrKa}/C2_{FeKa}$  can be obtained from the iron intensity  $C2_{FeKa}$  and chromium intensity  $C2_{CrKa}$  at the center thickness point of the inner oxide layer **2**. Furthermore, peak intensity ratio of chromium to iron  $R3=C3_{CrKa}/C3_{FeKa}$  can be obtained from the 20 iron intensity  $C3_{FeKa}$  and chromium intensity  $C3_{CrKa}$  at the center thickness point of the outer oxide layer **3**.

As for the base material using a soft magnetic alloy for electronic components as proposed by the present invention, the grain is coated by, of the oxide layers in the two-layer 25 structure, the inner oxide layer produced on the surface of the grain **1**, while the outer oxide layers of such grains **1** are inter-bonded (refer to FIG. 2(A)). Under the present invention, the coating of adjacent grains **1** by the inner layers **2** of the two-oxide-layer structures produced on the surfaces of the 30 grains **1**, and inter-bonding of the outer oxide layers **3**, manifest as improved magnetic characteristics and strength of the base material using the soft magnetic alloy for electronic component. As mentioned in detail later, the oxide layer in the present invention is produced on the surface of the grain **1** by 35 agitating and mixing grains **1** and thermoplastic resin or other binder, compression-molding the obtained pellets, and then heat-treating the molded product, where, if the molding pressure is raised, the grains **1** are inter-bonded directly without involving any oxide layer (refer to FIG. 2(B)) as confirmed 40 from the result of SEM observation. In addition, the outer surface layer of the oxide layer not involved in the inter-bonding of soft magnetic alloy grains has irregularities and the specific surface area of grains increases compared to before the heat treatment, which has the effect of improving 45 the insulation property further.

To manufacture the base material using a soft magnetic alloy for electronic components as proposed by the present invention, one embodiment is to add thermoplastic resin or other binder to the material grain containing chromium, silicate and iron and then agitate and mix the ingredients to 50 obtain pellets first. Next, these pellets are compression-molded to form a molded product, and the obtained molded product is heat-treated in air at 500 to 900° C. This heat treatment in air removes the thermoplastic resin that has been mixed in, and produces a metal oxide layer on the grain surface by bonding the chromium, which was originally present in the grain and has migrated to the surface due to heat treatment, and the iron, which is a main ingredient of the grain, with oxygen, while at the same time the oxide layers on 55 adjacent grains are inter-bonded. The oxide layer (metal oxide layer) has a two-layer structure constituted by an inner layer which is produced on the alloy grain surface and whose main ingredient is chromium oxide, and an outer layer which is present on the outer side of the inner layer and whose main 60 ingredient is an oxide containing iron and chromium offering higher specific resistance, where the outer layer is formed thicker than the inner layer. Since the surface of soft magnetic 65

grains is coated by inner layers and at least some soft magnetic grains are inter-bonded via outer layers, a base material using a soft magnetic alloy for electronic components, which ensures insulation between the grains, can be provided. Examples of material grain include grains manufactured by the water atomization method, while examples of the shape of the material grain include spherical and flat shapes.

Under the present invention, raising the heat treatment temperature in the oxygen ambience breaks down the binder, causing the soft magnetic alloy to be oxidized. For the heat treatment conditions for molded product to form the aforementioned oxide layer having a two-layer structure, it is desirable to raise the temperature in air to around 500 to 900° C. at a rate of 30 to 300° C./hour and then hold this temperature for another 1 to 10 hours. By implementing the heat treatment at temperatures and rates of rise in temperature in these ranges, the aforementioned superior two-oxide-layer structure can be formed. More preferably the heat treatment can be implemented at 600 to 800° C. It can also be implemented in conditions other than in air, such as in an ambience whose partial oxygen pressure is equivalent to that in air. In a reducing ambience or non-oxidizing ambience, heat treatment does not produce metal oxide layer, and consequently the grains are sintered together and volume resistivity drops significantly. Although the oxygen concentration and water vapor amount in the ambience are not specifically limited, air or dry air is desired from the production viewpoint. If the heat treatment temperature exceeds 500° C., excellent strength and excellent volume resistivity can be obtained. If the heat treatment temperature exceeds 900° C., on the other hand, strength increases but the volume resistivity drops. Furthermore, if the rate of rise in temperature exceeds 300° C./hour, the two-oxide-layer structure cannot be obtained and there will be only a single oxide layer.

Due to the heat treatment, the surface of the oxide layer that grows around the grain 1 always has irregularities, where these irregularities become more prominent when the rate of rise in temperature is lower, and absorbed in areas where the grains are inter-bonded via their outer oxide layers, but remain in areas where oxide layers are not involved in the bonding (oxide layers adjacent to voids). These irregularities formed on the grain surface increase the surface resistance and improve the insulation property further.

In addition, by setting the retention time at the above heat treatment temperature to 1 hour or more, outer oxide layers 3 are formed easily from a metal oxide containing iron and chromium. Although the specific maximum limit of holding time is not set because the oxide layer thickness saturates at a certain value, a period of 10 hours or less is appropriate from the production viewpoint. Furthermore, the temperature may be held at a certain level during the course of raising the temperature at the aforementioned rate. If the heat treatment temperature is 700° C., for example, it is possible to raise the temperature to around 500 to 600° C. at the aforementioned rate and then hold that temperature for 1 hour, after which the temperature is raised further to 700° C. at the aforementioned rate. As mentioned above, use of heat treatment conditions within the aforementioned ranges achieves excellent strength and excellent volume resistivity at the same time in the process of obtaining a base material using a soft magnetic alloy having an oxide layer. In other words, formation of in-grain crystal grains and oxide layers is controlled by the heat treatment temperature, heat treatment time, oxygen amount in the heat treatment ambience, etc.

For the soft magnetic alloy base material for electronic component as proposed by the present invention, high magnetic permeability and high saturated magnetic flux density

can be obtained by applying the above process to iron-silicate-chromium alloy powder. By this high magnetic permeability, an electronic component which is smaller than conventional components but accepts current larger than possible with conventional components can be obtained. In addition, no resin or glass is used, which is different from those coil components made of soft magnetic alloy grains bonded by resin or glass, meaning that no high molding pressure is needed and production cost can be kept low. Furthermore, with the soft magnetic alloy base material for an electronic component in this embodiment, high saturated magnetic flux density is maintained and glass component, etc., will not appear on the material surface even after the heat treatment in air, and consequently a compact chip-type electronic component having high dimensional stability can be provided.

Next, the first embodiment of an electronic component conforming to the present invention is explained by referring to FIGS. 1, 2, 3 and 4. FIGS. 1 and 2 are not explained here, because they were already explained in connection with the earlier embodiment of base material using a soft magnetic alloy for an electronic component. FIG. 3 is a side view, with partial perspective projection, of the electronic component in this embodiment. FIG. 4 is a longitudinal section view showing the internal structure of the electronic component in this embodiment. The electronic component 20 in this embodiment is a coil-type electronic component, or specifically a winding-type chip inductor. It is comprised of a drum-type core 11 constituting the above base material 10 using a soft magnetic alloy for an electronic component, and the aforementioned base material 10, and has a pair of sheet-shaped cores 12, 12, which are not illustrated, connecting the two flange parts 11b, 11b of the drum-type core 11. On the installation surfaces of the flange parts 11, 11b of the core 11, a pair of external conductive films 14, 14 are formed, respectively. Also, a coil 15 constituted by an insulation coated conductive wire is wound around the winding center 11a of the core 11 to form a winding part 15a, while both ends 15b, 15b are thermo-compression-bonded to the external conductive films 14, 14 on the installation surfaces of the flange parts 11b, 11b, respectively. The external conductive films 14, 14 each have a baked conductive layer 14a formed on the surface of the base material 10, as well as a Ni plating layer 14b and Sn plating layer 14c that are layered on top this baked conductive layer 14a. The aforementioned sheet-shaped cores 12, 12 are bonded by resin adhesive to the flange parts 11b, 11b of the drum-type core 11.

The electronic component 20 in this embodiment has: multiple grains containing chromium, silicon and iron; an oxide layer formed on the surface of these grains, wherein this oxide layer contains at least iron and chromium and whose peak strength ratio of chromium relative to iron is higher than the peak strength ratio of chromium relative to iron in the aforementioned grain, based on calculation by the ZAF method through energy diffusion X-ray analysis using a scanning electron microscope; and a base material 10, as a core 11, which uses the aforementioned soft magnetic alloy for an electronic component where oxide layers formed on the surfaces of the aforementioned grains adjacent to one another are bonded. At least a pair of external conductive layers 14, 14 are formed on the surface of the base material 10. The base material 10 using a soft magnetic alloy for the electronic component, which constitutes the electronic component 20 in this embodiment, is not explained here because it has already been explained earlier.

The core 11 at least has a winding center 11a, where the cross-section of the winding center 11a may be sheet-shaped (rectangular), circular, or oval. Also, it is desirable that at least

## 11

one flange part **11** is provided on one end of the aforementioned winding center **11a**. With a flange part **11**, the coil position relative to the winding center **11a** can be controlled easily using the flange part **11**, to help stabilize characteristics such as inductance and the like. The core **11** can be embodied in several ways, such as an embodiment with one flange part, embodiment with two flange parts (drum core), embodiment where the long-axis direction of the winding center **11a** is placed vertically to the installation surface, and embodiment where the long-axis direction is placed horizontally to the installation surface. Especially, an embodiment where a flange part is provided only on one axial end of the winding center **11a** and the long-axis direction of the winding center **11a** is placed vertically to the installation surface, is preferable in reducing the height.

The external conductive film **14** is formed on the surface of the base material **10** using a soft magnetic alloy for an electronic component, and an end of the coil is connected to the external conductive film **14**. The external conductive film **14** may be a baked conductive film or resin conductive film. A baked conductive film can be formed on the base material **10** using a soft magnetic alloy for an electronic component by, for example, baking a paste made of silver to which glass has been added at a specified temperature. A resin conductive film can be formed on the base material **10** using a soft magnetic alloy for an electronic component by, for example, applying a paste containing silver and epoxy resin and then treating the paste at a specified temperature. In the case of baked conductive film, heat treatment can be applied after the conductive film has been formed.

The coil may be made of copper or silver. Desirably the coil is given insulation coating. The coil may be a rectangular wire, angular wire, or rounded wire. Use of a rectangular or angular wire is desirable because the gaps between windings can be reduced and the electronic component can be kept small.

A specific example of forming the baked conductive layer **14a** that constitutes the conductive films **14**, **14** on the surface of the base material **10** using a soft magnetic alloy for an electronic component in the electronic component **20** in this embodiment, is given below. Bake-type electrode material paste containing metal grains and glass frit (bake-type Ag paste is used in this example) is applied on the installation surfaces of the flange parts **11b**, **11b** of the base material **10**, or core **11**, and then heat treatment is given in the standard atmosphere to sinter and affix the electrode material directly on the surface of the base material **10**. Ni and Sn metal plating layers may also be formed, by means of electrolysis, on the surface of the baked conductive layer **14a** that has been formed.

The electronic component **20** in this embodiment can also be obtained by the manufacturing method explained below. Material containing material grains and binder is molded, where the specific composition of material grains is, say, 2 to 8 percent by weight of chromium, 1.5 to 7 percent by weight of silicon and 88 to 96.5 percent by weight of iron, and bake-type electrode material paste containing metal powder and glass frit is applied on the surface of the obtained molded product at least over an area that will become the installation surface, and the resulting molded product is heat-treated at 400 to 900° C. in the standard atmosphere. Metal plating layers may also be formed on the baked conductive layer that has been formed. According to this method, an oxide layer is generated on the surface of grains, and a base material using a soft magnetic alloy for an electronic component where oxide layers on the surfaces of adjacent grains are bonded with one another can be formed simultaneously with a baked

## 12

conductive layer constituting the conductive film on the surface of this base material, which simplifies the manufacturing process. Since chromium oxidizes more easily than iron, excessive oxidization of iron can be prevented when heat is applied in an oxidizing atmosphere, compared to pure iron.

Next, an example of variation of the embodiment of the base material using a soft magnetic alloy for an electronic component under the present invention is explained by referring to FIG. 5. FIG. 5 is a perspective view of internal structure, showing an example of variation of the base material **10'** using a soft magnetic alloy for an electronic component. The base material **10'** in this example of variation has a rectangular solid appearance, while on the inside an internal coil **35** wound in helical manner is buried and the pullout parts at both ends of the internal coil **35** are exposed to a pair of opposing end faces of the base material **10'**. The base material **10'**, together with the internal coil **35** buried inside, constitutes a laminated chip **31**. Just like the base material **10** using a soft magnetic alloy for the electronic component in the first embodiment described earlier, the base material **10'** using a soft magnetic alloy for the electronic component in this example of variation is also characterized in that it has: multiple grains containing chromium, silicon, and iron; an oxide layer formed on the surface of these grains, wherein this oxide layer contains at least iron and chromium and whose peak strength ratio of chromium relative to iron is higher than the peak strength ratio of chromium relative to iron in the grain, based on energy diffusion X-ray analysis using a scanning electron microscope, and wherein oxide layers formed on the surfaces of adjacent grains are bonded with one another. The base material **10'** using a soft magnetic alloy for the electronic component in this example of variation also has the same operations and effects as those of the base material **10** using a soft magnetic alloy for the electronic component in the first embodiment described earlier.

Next, an example of variation of the embodiment of an electronic component under the present invention is explained by referring to FIG. 6. FIG. 6 is a perspective view of internal structure, showing an electronic component **40** being an example of variation. The electronic component **40** in this example of variation is constituted by the base material **10'** using a soft magnetic alloy for the electronic component described in the aforementioned example of variation, where a pair of external conductive films **34**, **34** are formed on or near a pair of opposing end faces of the base material in a manner connecting the exposed pullout parts of the internal coil **35**. These external conductive films **34**, **34**, while not illustrated, have a baked conductive layer and an Ni plating layer and an Sn plating layer that are layered on top of this baked conductive layer, just like the external conductive layers **14**, **14** of the electronic component **20** in the first embodiment described earlier.

In addition, it is desirable that the multiple grains constituting the base material using a soft magnetic alloy for an electronic component, as proposed by the present invention, should have a composition of “2 percent by weight≤Chromium≤8 percent by weight,” “1.5 percent by weight≤Silicon≤7 percent by weight” and “88 percent by weight≤Iron≤96.5 percent by weight.” When the respective components are within these ranges, the base material using a soft magnetic alloy for an electronic component as proposed by the present invention demonstrates even higher strength and higher volume resistivity. In general, soft magnetic alloys containing larger amounts of Fe have higher saturation magnetic flux densities and thereby offering better DC superimposition characteristics. However, higher Fe contents mean generation of rust in a condition of high temperature and

## 13

humidity, which causes various problems in use, such as shedding of rusted material. It is a well-known fact that adding chromium to magnetic alloys is effective in raising the corrosion resistance of alloys, one representative example of which is stainless steel. However, when compacted powder magnetic cores were made from such magnetic alloy powder containing chromium by applying heat treatment in a non-oxidizing atmosphere, specific resistances measured by an insulation resistance tester were around  $10^{-1}$   $\Omega$ cm, which is enough to prevent eddy-current loss between grains, but short of  $10^5$   $\Omega$ cm or more needed to form an external conductive film, and as a result no metal plating layer could be formed on the baked conductive layer constituting the external conductive film.

Accordingly, under the present invention, a molded product containing a binder and material grains having the aforementioned composition is heat-treated under certain conditions in an oxidizing atmosphere to generate on the surface of grains a two-layer structure oxide layer constituted by a metal oxide layer, while covering the surface of the grains by the inner layer of the oxide layer and causing at least a portion of the oxide layer on the surface of adjacent grains to be bonded with one another by the outer layer of the oxide layer, to achieve high strength. The base material using a soft magnetic alloy for an electronic component, thus obtained, had a greatly improved volume resistivity  $\rho_v$  of  $10^5$   $\Omega$ cm or more, which made it possible to form plating layers of metal such as Ni, Sn and the like, without causing plating extension, on the baked conductive layer constituting the external conductive film formed on the surface of the base material.

The reason the composition is limited for the base material using a soft magnetic alloy for an electronic component, in a more favorable form of the present invention, is explained. If the chromium content in the composition of multiple grains is less than 2 percent by weight, the volume resistivity becomes low and no metal plating layer can be formed, without causing plating extension, on the baked conductive layer constituting the external conductive film.

If chromium is contained by more than 8 percent by weight, the volume resistivity also becomes low and no metal plating layer can be formed, without causing plating extension, on the baked conductive layer constituting the external conductive film. If an oxide coat is formed using Fe—Si—Al powder via heat treatment in the standard atmosphere, as described in Patent Literature 1 above, the coat is constituted by a chromium-free oxide. As a result, its volume resistivity becomes lower than  $10^5$   $\Omega$ cm and no metal plating layer can be formed, without causing plating extension, on the baked conductive layer constituting the external conductive film.

With the above base material using a soft magnetic alloy for an electronic component, Si in the composition of multiple grains has the effect of improving the volume resistivity, but this effect is not achieved when the content is less than 1.5 percent by weight, while the achieved effect is not sufficient when the content is more than 7 percent by weight, and the volume resistivity is also less than  $10^5$   $\Omega$ cm, which means that no metal plating layer can be formed, without causing plating extension, on the baked conductive layer constituting the external conductive film. Si also has the effect of improving the magnetic permeability, but if the content is more than 7 percent by weight, a relative decrease in Fe content causes the saturation magnetic flux density to drop. It also results in lower moldability, which is another factor that lowers the magnetic permeability and the saturation magnetic flux density.

With the above base material using a soft magnetic alloy for an electronic component, the saturation magnetic flux

## 14

density drops, while moldability also drops to decrease the magnetic permeability and saturation magnetic flux density, if the iron content in the composition of multiple grains is less than 88 percent by weight. If the iron content is more than 96.5 percent by weight, the volume resistivity drops due to a relative drop in chromium content and silicon content.

Under the present invention, it is also desirable that the average size of multiple grains is 5 to 30  $\mu$ m in equivalent average grain size  $d_{50\%}$  (arithmetic mean) of material grains. 10 Also note that the average size of multiple grains mentioned above can be approximated by a value obtained by capturing a composition image of a cross-section of the base material using a scanning electron microscope (SEM) at a magnification of 3000 times, and then dividing the total sum of simple 15 averages  $D = (d_1 + d_2)/2$  of grains whose cross-section outline can be fully observed, by the total number of grains, where  $d_1$  and  $d_2$  represent the long-axis dimension and short-axis dimension of the cross-section of each grain, respectively.

The group of alloy metal grains has a granular distribution, 20 and grains are not necessarily circular but have irregular shapes instead. When solid alloy metal grains are observed two-dimensionally (on a plane), their size varies depending on which cross-section is observed. Accordingly, under the present invention, the average grain size is evaluated by measuring more grains. In this sense, it is desirable to measure at least 100 applicable grains under the conditions specified below. The specific method is as follows. First the largest diameter of the grain cross-section represents the long axis, and the point that equally divides the length of the long axis is 25 obtained. Next, the smallest diameter of the grain cross-section that includes this point represents the short axis. The two are defined as the long-axis dimension and short-axis dimension, respectively. Grains to be measured are arranged sequentially from the one having the largest diameter of its 30 cross-section, and measurement is performed until the cumulative ratio of grain cross-sections accounts for 95% of all area shown in the scanning electron microscope (SEM) image excluding grains whose cross-section outline is cannot be 35 fully observed, voids, and oxide layers. As long as the average grain size mentioned above is within the specified range, high 40 saturation magnetic flux density (1.4 T or more) and high magnetic permeability (27 or more) can be obtained, and generation of eddy-current loss in the grain can be prevented even at frequencies of 100 kHz and above. In the present 45 disclosure, disclosed numeral numbers refer to approximate numbers in some embodiments, and the upper and lower endpoints of described ranges are included in some embodiments, or excluded in some embodiments. Further, in some 50 embodiments, numeral numbers refer to average numbers, representative numbers, median, etc.

## EXAMPLES

The following explains the present invention in greater 55 detail using examples and a comparative example. It should be noted, however, that the present invention is not at all limited to these examples and the comparative example.

To determine the level of magnetic characteristics of each 60 base material using a soft magnetic alloy for an electronic component, grain materials were molded into a toroidal shape of 14 mm in outer diameter, 8 mm in inner diameter and 3 mm in thickness by adjusting the molding pressure to between 6 and 12 tons/cm<sup>2</sup> so that the fill ratio of material grains would become 80 percent by volume, after which the molded product 65 was heat-treated in the standard atmosphere and a coil constituted by urethane-coated copper wire of 0.3 mm in diameter was wound around the obtained base material by 20

## 15

turns to obtain a test sample. Magnetic permeability  $\mu$  was measured with an L chromium meter (4285A manufactured by Agilent Technologies) at a measurement frequency of 100 kHz. Samples whose saturation magnetic flux density  $B_s$  was 0.7 T or more were considered of good quality.

To determine the level of strength of each base material using a soft magnetic alloy for an electronic component, 3-point bending rupture stress was measured, as follows, according to the measurement method illustrated in FIG. 7. Each test piece used for measurement of 3-point bending rupture stress was prepared by molding material grains into a sheet shape of 50 mm in length, 10 mm in width and 4 mm in thickness by adjusting the molding pressure to between 6 and 12 tons/cm<sup>2</sup> so that the fill ratio of material grains would become 80 percent by volume, and then heat-treating the molded product in the standard atmosphere.

In addition, to determine the level of volume resistivity of each base material using a soft magnetic alloy for an electronic component, measurement was performed, as shown in FIG. 8, according to JIS-K6911. Each test piece used for measurement of volume resistivity was prepared by molding material grains into a disk shape of 100 mm in diameter and 2 mm in thickness by adjusting the molding pressure to between 6 and 12 tons/cm<sup>2</sup> so that the fill ratio of material grains would become 80 percent by volume, and then heat-treating the molded product in the standard atmosphere.

## Example 1

For the material grains to obtain a base material using a soft magnetic alloy for an electronic component, alloy powder (PF-20F manufactured by Epson Atmix K.K.) was used which is a type of water-atomized powder whose average grain size (d50%) is 10 $\mu$  and composition ratio was 5 percent by weight of chromium, 3 percent by weight of silicon and 92 percent by weight of iron. The average grain size d50% of material grains described above was measured using a granularity analyzer (9320HRA manufactured by Nikkiso). Each of the above grains was polished until its cross-section in a thickness direction cutting across roughly the center of the grain was exposed, and the obtained cross-section was captured with a scanning electron microscope (SEM: S-4300SE/N manufactured by Hitachi High-Technologies) at a magnification of 3000 times to obtain a composition image, which was then used to calculate the composition near the center of the grain and also near the surface by the ZAF method through energy diffusion X-ray analysis (EDS), confirming that the above composition ratio near the center of the grain was roughly the same as the corresponding composition ratio near the surface. Next, the above grains were mixed with polyvinyl butylal (S-LEC BL, a solution with a solid concentration of 30 percent by weight, manufactured by Sekisui Chemical) using a wet-type rolling agitator to obtain pellets. The obtained pellets were molded into an angular sheet shape of 50 mm in length, 10 mm in width, and 4 mm in thickness; a disk shape of 100 mm in diameter and 2 mm in thickness; a toroidal shape of 14 mm in outer diameter, 8 mm in inner diameter, and 3 mm in thickness; a drum-type core having angular flange parts (1.6 mm wide $\times$ 0.6 mm high $\times$ 0.3 mm thick) at both ends of winding core parts (1.0 mm wide $\times$ 0.36 mm high $\times$ 1.4 mm long); and a pair of sheet-shaped cores (2.0 mm long $\times$ 0.5 mm wide $\times$ 0.2 mm thick), by setting a molding pressure at 8 tons/cm<sup>2</sup> so that the fill ratio of multiple grains would become 80 percent by volume. The disk-shaped molded product, toroidal molded product, drum-type molded product and pair of sheet-shaped molded products, as

## 16

obtained above, were heated to 700°C. at a heating-up rate of 100°C./hour and heat-treated for 3 hours in the standard atmosphere.

The disk-shaped base material obtained by heat-treating the above disk-shaped molded product was measured for magnetic permeability  $\mu$ , 3-point bending rupture stress, and volume resistivity according to JIS-K6911, and the result is shown in Table 1. Also, the drum-type base material obtained by heat-treating the above drum-type molded product was polished until its cross-section in thickness direction cutting across roughly the center of the winding center was exposed, and the obtained cross-section was captured with a scanning electron microscope (SEM) at a magnification of 3000 times to obtain a composition image. Next, pixels of the composition image obtained above were classified into four contrast levels. The contrast ranks were determined in such a way that, among the grains shown in the above composition image whose cross-section outline could be fully observed, those whose simple average size  $D=(d_1+d_2)/2$  was greater than the average grain size of material grains (d50%), where d1 and d2 represent the long-axis dimension and short-axis dimension of the cross-section of each grain, respectively, were deemed to be of the reference brightness rank of composition contrast, and any part of the above composition image corresponding to this brightness rank was judged as a grain 1. On the other hand, any part whose composition contrast was next darker than the above reference brightness rank was judged as an outer layer of an oxide layer 3, and any part whose contrast was further darker than the above was judged as an inner layer of an oxide layer 2. In addition, any part whose contrast was the darkest was judged as a void 3 (not shown). The obtained result confirms that the outer layer 3 of the oxide layer formed on the surface of the adjacent grains 1 was bonded with one another.

Next, among the grains shown in this composition image whose cross-section outline could be fully observed, a grain whose simple average size  $D=(d_1+d_2)/2$  was greater than the average grain size of material grains (d50%), where d1 and d2 represent the long-axis dimension and short-axis dimension of the cross-section of each grain, respectively, was extracted and the composition near the point of intersection of its long axis and short axis was calculated by the ZAF method through energy diffusion X-ray analysis (EDS). The result was then compared against the composition ratio of the above material grain to confirm that the composition ratio of multiple grains constituting the above base material was roughly or substantially the same as the composition ratio of material grains.

Next, the composition of the point of intersection between the long axis d1 and short axis d2 in the grain 1 was obtained on the aforementioned composition image by SEM-EDS. Next, the composition at the center thickness point of the oxide layer at a location whose oxide layer thickness corresponds to the average thickness of the maximum thickness t1 and minimum thickness t2 of the oxide layer on the surface of the grain 1, calculated by  $T=(t_1+t_2)/2$ , was obtained by SEM-EDS on the aforementioned composition image.

From the above results, the soft magnetic alloy base material for the electronic component in Example 1 was confirmed to have multiple grains 1 containing 5 percent by weight of chromium, 3 percent by weight of silicate, and 92 percent by weight of iron, and a two-oxide-layer structure produced on the surface of each grain 1, where the inner oxide layer 2 contained chromium oxide as its main ingredient and had an average thickness of 40 nm, while the outer oxide layer 3 contained iron-chromium oxide as its main ingredient and had an average thickness of 70 nm.

The obtained results are shown in Table 1. As shown, good measurement results were obtained, such as 55 in magnetic permeability  $\mu$ , 14 kgf/mm<sup>2</sup> in base material strength (rupture stress),  $4.2 \times 10^7$   $\Omega\cdot\text{cm}$  in volume resistivity. Next, a coil made of insulated sheathed conductive wire was wrapped around the winding core of the aforementioned drum-type base material and both ends of the coil were thermally bonded to the external conductive film, respectively, and a sheet-shaped base material obtained by heat-treating the aforementioned sheet-shaped molded product was bonded by resin adhesive to both sides of the flange part of the drum-type base material, to obtain a winding-type chip inductor.

#### Example 2

An evaluation sample was prepared in the same manner as in Example 1, except that the composition ratio of the material grain was changed to 3 percent by weight of chromium, 5 percent by weight of silicate, and 92 percent by weight of iron. The obtained results are shown in Table 1. As shown in Table 1, good measurement results were obtained, just as in Example 1, such as 50 in magnetic permeability  $\mu$ , 9 kgf/mm<sup>2</sup> in base material strength (rupture stress), and  $2.0 \times 10^7$   $\Omega\cdot\text{cm}$  in volume resistivity. SEM observation and SEM-EDS analysis, performed in the same manner as in Example 1, also confirmed that the metal oxide (oxide layer) formed on the grain surface due to heat treatment had a two-layer structure constituted by an inner layer 2 (average thickness: 30 nm) formed by chromium oxide and an outer layer 3 (average thickness: 66 nm) formed by iron-chromium oxide, with the outer oxide layers 3 bonding together.

#### Example 3

An evaluation sample was prepared in the same manner as in Example 1, except that the composition ratio of the material grain was changed to 6 percent by weight of chromium, 2 percent by weight of silicate and 92 percent by weight of iron. The obtained results are shown in Table 1. As shown in Table 1, good measurement results were obtained, just as in Example 1, such as 46 in magnetic permeability  $\mu$ , 14 kgf/mm<sup>2</sup> in base material strength (rupture stress), and  $7.0 \times 10^6$   $\Omega\cdot\text{cm}$  in volume resistivity. SEM observation and SEM-EDS analysis, performed in the same manner as in Example 1, also confirmed that the metal oxide (oxide layer) formed on the grain surface due to heat treatment had a two-layer structure constituted by an inner layer 2 (average thickness: 50 nm) formed by chromium oxide and an outer layer 3 (average thickness: 80 nm) formed by iron-chromium oxide, with the outer oxide layer 3 bonding together.

#### Example 4

An evaluation sample was prepared in the same manner as in Example 1, except that the composition ratio of the material grain was changed to 6 percent by weight of chromium, 4 percent by weight of silicate and 94 percent by weight of iron. The obtained results are shown in Table 1. As shown in Table 1, good measurement results were obtained, just as in Example 1, such as 48 in magnetic permeability  $\mu$ , 14 kgf/mm<sup>2</sup> in base material strength (rupture stress), and  $8.0 \times 10^6$   $\Omega\cdot\text{cm}$  in volume resistivity. SEM observation and SEM-EDS

analysis, performed in the same manner as in Example 1, also confirmed that the metal oxide (oxide layer) formed on the grain surface due to heat treatment had a two-layer structure constituted by an inner layer 2 (average thickness: 40 nm) formed by chromium oxide and an outer layer 3 (average thickness: 75 nm) formed by iron-chromium oxide, with the outer oxide layers 3 bonding together.

#### Example 5

An evaluation sample was prepared in the same manner as in Example 1, except that the composition ratio of the material grain was changed to 4 percent by weight of chromium, 2 percent by weight of silicate and 89 percent by weight of iron. The obtained results are shown in Table 1. As shown in Table 1, good measurement results were obtained, just as in Example 1, such as 47 in magnetic permeability  $\mu$ , 18 kgf/mm<sup>2</sup> in base material strength (rupture stress), and  $5.1 \times 10^5$   $\Omega\cdot\text{cm}$  in volume resistivity. SEM observation and SEM-EDS analysis, performed in the same manner as in Example 1, also confirmed that the metal oxide (oxide layer) formed on the grain surface due to heat treatment had a two-layer structure constituted by an inner layer 2 (average thickness: 35 nm) formed by chromium oxide and an outer layer 3 (average thickness: 70 nm) formed by iron-chromium oxide, with the outer oxide layers 3 bonding together.

#### Example 6

An evaluation sample was prepared in the same manner as in Example 1, except that the molding pressure was changed to 12 tons/cm<sup>2</sup>. The obtained measurement results are shown in Table 1. As shown in Table 1, good measurement results were obtained, just as in Example 1, such as 59 in magnetic permeability  $\mu$ , 15 kgf/mm<sup>2</sup> in base material strength (rupture stress), and  $4.2 \times 10^5$   $\Omega\cdot\text{cm}$  in volume resistivity. SEM-EDS analysis, performed in the same manner as in Example 1, also confirmed that the metal oxide (oxide layer) formed on the grain surface due to heat treatment had a two-layer structure constituted by an inner layer 2 (average thickness: 35 nm) formed by chromium oxide and an outer layer 3 (average thickness: 65 nm) formed by iron-chromium oxide. In addition, SEM observation performed in the same manner as in Example 1 found a presence of grains inter-bonded directly without involving any oxide layer. This is probably due to the higher molding pressure that increased the contact area between grains.

#### Comparative Example 1

An evaluation sample was prepared in the same manner as in Example 1, except that the rate of rise in temperature during heat treatment was changed to 400° C./hour. The obtained measurement results are shown in Table 1. As shown in Table 1, the magnetic permeability  $\mu$  was 45, base material strength (rupture stress) was 7.4 kgf/mm<sup>2</sup>, volume resistivity was  $4.2 \times 10^5$   $\Omega\cdot\text{cm}$ , none of which was better than the measurement results of Examples 1 to 6. In addition, SEM observation and SEM-EDS analysis performed in the same manner as in Example 1 confirmed that, although grains were inter-bonded via metal oxides (oxide layers) formed on their surface due to heat treatment, the oxide layers had only a single layer of iron-chromium oxide.

TABLE 1

|                          | Composition<br>(percent by weight) |    |    | Rupture<br>stress | Volume<br>resistivity | Outer layer<br>thickness | Inner layer<br>thickness |    |
|--------------------------|------------------------------------|----|----|-------------------|-----------------------|--------------------------|--------------------------|----|
|                          | Cr                                 | Si | Fe | $\mu$             | kgf/mm <sup>2</sup>   | $\Omega \cdot \text{cm}$ | nm                       | nm |
| Example 1                | 5                                  | 3  | 92 | 55                | 14                    | $4.2 \times 10^7$        | 70                       | 40 |
| Example 2                | 3                                  | 5  | 92 | 50                | 9                     | $2.0 \times 10^7$        | 66                       | 30 |
| Example 3                | 6                                  | 2  | 92 | 46                | 14                    | $7.0 \times 10^6$        | 80                       | 50 |
| Example 4                | 6                                  | 4  | 94 | 48                | 14                    | $8.0 \times 10^6$        | 75                       | 40 |
| Example 5                | 4                                  | 2  | 89 | 47                | 18                    | $5.1 \times 10^5$        | 70                       | 35 |
| Example 6                | 5                                  | 3  | 92 | 59                | 15                    | $4.2 \times 10^5$        | 65                       | 35 |
| Comparative<br>example 1 | 5                                  | 3  | 92 | 45                | 7.4                   | $4.2 \times 10^5$        | —                        | —  |

A soft magnetic alloy base material for an electronic component according to the present invention, and an electronic component using such base material, are suitable for a compact electronic component that can be surface-mounted on a circuit board. In particular, they are suitable for size reduction of power inductor components through which high current flows.

In the present disclosure where conditions and/or structures are not specified, a skilled artisan in the art can readily provide such conditions and/or structures, in view of the present disclosure, as a matter of routine experimentation. Also, in the present disclosure including the examples described above, any ranges applied in some embodiments may include or exclude the lower and/or upper endpoints, and any values of variables indicated may refer to precise values or approximate values and include equivalents, and may refer to average, median, representative, majority, etc. in some embodiments. Further, in this disclosure, an article "a" may refer to a species or a genus including multiple species, and "the invention" or "the present invention" may refer to at least one of the embodiments or aspects explicitly, necessarily, or inherently disclosed herein. In this disclosure, any defined meanings do not necessarily exclude ordinary and customary meanings in some embodiments.

The present application claims priority to Japanese Patent Application No. 2011-236947, filed Oct. 28, 2011, the disclosure of which is incorporated herein by reference in its entirety. In some embodiments, as the soft magnetic alloy grains, for example, those disclosed in U.S. Patent Application Publication No. 2011/0267167, No. 2012/0038449, No. 2012/0188049, and No. 2012/0188046 can be used, each disclosure of which is incorporated herein by reference in its entirety.

15 It will be understood by those of skill in the art that numerous and various modifications can be made without departing from the spirit of the present invention. Therefore, it should be clearly understood that the forms of the present invention are illustrative only and are not intended to limit the scope of the present invention.

We claim:

25 1. A coil-type electronic component having a coil inside or on the surface of a base material, wherein the base material is constituted by a group of soft magnetic alloy grains whose main ingredients are iron, silicate and chromium, and an oxide layer having a two-layer structure is formed on the surface of each soft magnetic alloy grain where, of the oxide layers in the two-layer structure, the inner layer is primarily 30 constituted by chromium oxide while the outer layer is primarily constituted by iron-chromium oxide, and the outer layers of soft magnetic alloy grains are inter-bonded, wherein, of the oxide layers in the two-layer structure, the outer layer is thicker than the inner layer.

35 2. A coil-type electronic component according to claim 1, wherein the surface of the outer oxide layer not bonding the soft magnetic alloy grains together has irregularities.

40 3. A coil-type electronic component according to claim 1, wherein the base material contains the soft magnetic alloy grains inter-bonded not via the oxide layers.

45 4. A coil-type electronic component according to claim 2, wherein the base material contains the soft magnetic alloy grains inter-bonded not via the oxide layers.

5. A coil-type electronic component according to claim 1, wherein the soft magnetic alloy grains are bonded without resin.

\* \* \* \* \*